

## UNITED STATES PATENT OFFICE

2,198,932

## LEAD ALLOY

François Cuveliez, Hoboken-lez-Anvers, Belgium,  
assignor to Société Générale Metallurgique de  
Hoboken, Hoboken - lez - Anvers, Belgium, a  
Belgian limited company

No Drawing. Original application August 2, 1938,  
Serial No. 222,670. Divided and this applica-  
tion February 9, 1939, Serial No. 255,509. In  
Great Britain October 15, 1937

## 1 Claim. (Cl. 75—167)

This application is a division of my application  
Ser. No. 222,670 filed August 2, 1938.

This invention relates to lead alloys to be used  
in the chemical industry.

5 A lead alloy according to the present invention  
is of the usual compact, non-porous, structure,  
and comprises from 0.3 to 13% Sb and from 0.2  
to 5% Hg.

Moreover, the alloy contains one or more of  
10 the metals Zn, Ca, Bi:

|    | Per cent                    |
|----|-----------------------------|
| Zn | 0 to 0.6                    |
| Ca | 0 to 0.1                    |
| Bi | 0 to 1, the rest being lead |

15 The non-porous alloys according to the present  
invention not only resist corrosion by chemical  
agents, more particularly of sulfuric acid and

nitrous gases, as is the case with sulfuric acid  
plants of the chamber method type, but in addition  
they have also a high resistance to mechanical  
and physical efforts.

The alloy according to the present invention 5  
has a compact structure, such as industrial alloys  
generally have when they are made by the known  
processes of casting, moulding or rolling.

I claim:

A compact lead alloy to be used more par- 10  
ticularly against corrosion by chemical agents,  
consisting of from 0.3 to 13% of antimony, from  
0.2 to 5% of mercury, from 0.1 to 0.6% of zinc,  
from 0.005 to 0.1% of calcium and from 0.2 to 1% 15  
of bismuth, the rest being lead.

FRANÇOIS CUVELIEZ.